

Nov. 23, 1937.

S. W. FERRIS ET AL

2,099,683

TREATMENT OF WAX MIXTURES

Filed Aug. 21, 1935

3 Sheets-Sheet 1

*Fig. 1*



Inventors  
Seymour W. Ferris  
Willard F. Houghton  
Henry C. Cowles, Jr.  
By J. Wallace Linne  
their Attorney

Nov. 23, 1937.

S. W. FERRIS ET AL

2,099,683

TREATMENT OF WAX MIXTURES

Filed Aug. 21, 1935

3 Sheets-Sheet 2

Fig. 2



Inventors  
Seymour W. Ferris  
Willard F. Houghton  
Henry C. Cowles, Jr.  
By *Wallace Gunn*  
their Attorney

Nov. 23, 1937.

S. W. FERRIS ET AL

2,099,683

TREATMENT OF WAX MIXTURES

Filed Aug. 21, 1935

3 Sheets-Sheet 3

*Fig. 3*



Inventors

Seymour W. Ferris  
Willard F. Houghton  
Henry C. Cowles, Jr.

By *J. Wallace Dunning*  
their Attorney

## UNITED STATES PATENT OFFICE

2,099,683

## TREATMENT OF WAX MIXTURES

Seymour W. Ferris, Aldan, Willard F. Houghton, Swarthmore, and Henry C. Cowles, Jr., Philadelphia, Pa., assignors to The Atlantic Refining Company, Philadelphia, Pa., a corporation of Pennsylvania

Application August 21, 1935, Serial No. 37,163

3 Claims. (Cl. 196—26)

The present invention relates to the treatment of solid or semi-solid waxy hydrocarbons, and relates more particularly to the separation of substantially oil-free waxy hydrocarbons derived from petroleum, and petroleum distillates or residues, into fractions having different physical properties.

An object of this invention is a process for the production of novel waxes or wax products from wax-bearing stocks or waxy hydrocarbon mixtures which have not heretofore been employed as a source of such novel wax products.

A further object of this invention is a process for the production of novel wax fractions which are substantially oil-free and differ from one another in melting point, crystal structure, hardness, plasticity and tackiness.

A further object of this invention is the production of novel wax fractions by sweating substantially oil-free waxy hydrocarbon mixtures obtained from hydrocarbon oils by methods other than sweating.

A further object of this invention is the production of novel wax fractions by sweating substantially oil-free waxy hydrocarbon mixtures other than commercial paraffin wax obtained from paraffin distillate by usual refining methods.

Briefly, our process consists in separating waxy hydrocarbon mixtures which have heretofore been considered as unsweatable, into substantially oil-free fractions having different physical properties, and particularly different refractive index-melting point relationships than waxes produced in accordance with the methods known and practiced by those skilled in the art. Our process involves the sweating of waxy hydrocarbon mixtures which have not heretofore been sweated, and more particularly our process is concerned with the separation of substantially oil-free waxy hydrocarbon mixtures into fractions by sweating.

It has been known that crude petroleums, and particularly those of the so-called paraffin-base or mixed-base types, contain certain hydrocarbons commonly known as paraffin wax. Such wax has been found to contain at least three fundamentally distinct crystalline types of wax, namely: plate, malocrystalline and needle waxes. Present refining methods, particularly sweating, have a tendency to remove the malocrystalline and needle type waxes with the oil, and leave as solid the plate type waxes, so that the finished waxes tend for the most part to approach toward the plate type. In the usual methods of refining crude petroleum, the crude is subjected to distillation thereby to separate it into a number of fractions of varying volatilities and viscosities. The fraction known as "paraffin distillate", which, in general, is a fraction having a boiling range of the order of from about 170° C. (340° F.) to

about 310° C. (590° F.), when distilled under an absolute pressure of 10 m. m. of mercury, and which ordinarily is obtained from paraffin base and mixed base crudes, is separated into a solid wax fraction and a liquid oil fraction by chilling and filter-pressing. The solid fraction or crude wax collected in the filter press is known as "slack wax", and contains a large quantity of oil. This oil is removed or reduced by subjecting the slack wax to a "sweating" operation which consists essentially in fractionally melting and draining the oil and lower melting waxes from higher melting waxes. The waxes resulting from the sweating operation are then further refined by any of the well-known processes, such as by treatment with sulphuric acid and/or percolation through fuller's earth. The products so obtained are the ordinary paraffin waxes of commerce, and are graded according to their melting points, into products differing in hardness and other properties. All of these products however, may, in general, be classed as hard and brittle, except at temperatures approaching their melting points; furthermore, they tend to crystallize rather coarsely.

After the paraffin distillate cut, usually there is separated from the crude during the distillation another higher boiling cut, known as the high viscosity fraction. This fraction also contains wax, but because of its particular crystalline form, it does not lend itself to separation directly by filter-pressing. Instead, this fraction is usually cold settled or centrifuged to effect a comparatively rough separation of the wax from the oil. The wax together with considerable oil, as it is separated by the cold settling or centrifuging operation, is known as "petrolatum stock", and contains a micro-crystalline form of wax generally known as "slop wax". Certain high melting waxes are occasionally obtained from "petrolatum stock" by repeated recrystallizations and settlings from naphtha solution. However, petrolatum stock cannot be successfully processed by either pressing or sweating. As a rule, the wax in petrolatum stock is not recovered, but is cracked or otherwise disposed of.

There are, in addition to the wax sources aforesaid, the residual stocks which contain a micro-crystalline wax, commonly known as petrolatum wax. This wax usually is not processed into a finished wax product, but becomes a slop wax, or in some cases, after separation is employed in the production of petroleum jellies or the like.

In the further treatment of slack wax from the filter press, as referred to above in connection with the processing of "paraffin distillates", the wax cake is melted and run into sweating pans, wherein it is cooled to a temperature substantially below its melting point, and thereafter heated to cause the oil occluded in the slack

wax to exude therefrom. The wax which is left after the first sweating is known as "crude scale" wax, and is usually resweated one or more times in the production of refined waxes. The oil which 5 exudes from this crude scale wax on resweating, carries with it some waxes which roughly may be designated as "wax intermediates". These waxes are to a large extent lost from the final 10 sweated wax products. Also, the oil passing from the wax in the first sweating, generally referred to as "foots" oil, carries with it substantial quantities of waxes which are in general not recovered.

It will be seen, therefore, that the usual methods 15 of wax recovery do not provide for the recovery of many waxes which may be of moderately high-melting point, but which because of their high solubility in the oil are sweated out with and retained in the oil.

20 We have discovered that waxes which by prior processes remain in the oil, as pointed out above, may be recovered and upon recovery have highly desirable properties. Further, we have succeeded in preparing a series of hydrocarbon waxes of 25 very desirable properties quite different from those of the hydrocarbon waxes heretofore known. These waxes may be prepared from "foots" oil, or intermediate waxes from the sweating operation, or from petrolatum stock or "slop 30 wax", or in short, from practically any oil which contains waxes lost by customary methods of wax recovery, of which methods those given above are typical.

It has been known heretofore to increase the 35 melting point of substantially oil-free commercial paraffin wax by sweating therefrom a portion of the lower melting waxes. It has likewise been known to obtain small quantities of paraffin wax from the "foots" oil resulting from the initial 40 sweating of paraffin slack wax, such process involving the concentration of low melting waxes by distilling a portion of the oil from the "foots" oil and thereafter sweating the resulting wax concentrate. Furthermore, it has been proposed 45 to obtain high melting wax from petrolatum wax containing on the order of 40% oil by distilling such wax to about 30% bottoms, diluting the distillate fraction with naphtha and filter pressing, and thereafter sweating the resulting press cake 50 containing on the order of 8%-10% oil to produce the high melting point wax.

Our process is distinguished from those of the prior art in that we sweat waxy hydrocarbon mixtures of a variety of types which have not heretofore been sweated, particularly substantially oil-free waxy hydrocarbons, to produce wax fractions having different physical properties. Moreover, the substantially oil-free wax fractions produced in accordance with our process 55 have a markedly different relationship between refractive index and melting point than oil-free waxes obtained from the resweating of commercial paraffin wax or wax mixtures derived from conventionally sweated paraffin slack wax.

60 In accordance with our invention, we may employ any method of preparing a substantially oil-free wax which does not involve sweating and consequent loss of desirable constituents, and thereafter subject the oil-free wax so prepared 65 to fractional separation by sweating. However, for a better understanding of our invention, we describe a specific method without intending to limit ourselves thereto.

According to the process set forth in a co-pending 70 application of S. W. Ferris, Serial No. 4157,

filed Jan. 29, 1935, we prepare an oil-wax mixture for example, by distillation, which upon cooling to the desired separating temperature will crystallize wax to the extent of substantially 10% or less of the total volume of the mixture; or we 5 dilute a wax-bearing stock with a suitable solvent, so that upon cooling to the desired separating temperature, wax will crystallize to the extent of 10% or less of the total volume of the mixture. The oil-wax mixture so prepared is then cooled 10 to the desired temperature, with or without agitation, in such a manner as to effect a dispersion of the wax crystals throughout the mother liquor with reasonable uniformity. If agitation is resorted to, the cooled mother liquor containing the 15 wax crystals is thereafter permitted to stand, un-agitated, for sufficient time to effect the formation of a highly porous wax mass, the structure of which has appreciable mechanical strength, such mass containing less than substantially 10% of 20 solid wax per unit volume of the mass. The displacement of the mother liquor from the cooled wax mass is then accomplished by passing a displacing liquid, preferably an oil solvent, through the mass in such a manner that a substantially 25 horizontal interface is maintained between the mother liquor in the mass and the displacing liquid, the displacement pressure (differential pressure or pressure drop through the wax mass) being of the order of 5 lbs./sq. in., or less per foot 30 depth of wax mass, and the concentration of crystalline wax being less than substantially 20% by volume of the mass in which mother liquor is still present. The displacement step is usually accompanied by the settling or compacting of 35 the wax mass from which the mother liquor is being removed, but such compacting is controlled to prevent the concentration of crystalline wax in the mass from exceeding substantially 20% by volume of the mass. This control is obtained by 40 the proper adjustment of the quantity of wax crystallized from the mother liquor to form the initial wax mass, the rate and degree of cooling, the differential pressure required for displacement and the gravity differentials between wax, 45 mother liquor and displacing liquid. Upon completion of the displacement operation the solvents employed may be separated from the oil and wax fractions by distillation.

In carrying out the process, it is necessary to 50 control the quantity of wax in the mother liquor so that the crystalline wax content of the mass resulting from the chilling of the mother liquor will not exceed substantially 10% of any unit volume of the mass at the beginning of the displacement operation. In most instances, it has been found that the crystalline wax contained in the wax mass at the beginning of the displacement step should be of the order of from 1% to 6% 55 by volume, and preferably of the order of from 2.5% to 4.5% by volume; it may, however, be as high as 10% by volume depending upon the character of the wax crystals. Furthermore, in general, the differential pressure required in effecting displacement does not exceed substantially 60 5 lbs./sq. in. per unit (1 foot) depth of the wax mass, and usually at the outset does not exceed 2 lbs./sq. in. It is to be understood, however, that at some stages of the operation, and particularly during the latter part thereof, the pressure may be somewhat in excess of 5 lbs./sq. in. per 65 1 foot depth of the mass. In accordance with the method above mentioned, we are able to prepare waxes containing less than 2% of oil, and in general, less than substantially 1% of oil. 70 75

*Example 1.*—Following the procedure above set forth, 35 parts by volume of a wax-bearing East Texas intermediate distillate having a Saybolt universal viscosity of 57 seconds at 210° F. and an A. P. I. gravity of 25.3° at 60° F., was admixed with 65 parts by volume of ethylene dichloride and heated to a temperature of about 120° F., until a homogeneous solution was obtained. This solution was chilled, with agitation, to a temperature of about 60° F., whereupon a portion of the wax crystallized to form a wax mass having the oil-solvent mixture containing uncryallized wax dispersed therethrough. The oil-solvent mixture or mother liquor was then displaced from the wax mass at a temperature of about 60° F., without substantial agitation and under a low differential pressure, by means of a wash liquid such as 88° A. P. I. petroleum naphtha. The washed wax, after removal therefrom of wash naphtha, by distillation, had an A. S. T. M. melting point of 153° F., a refractive index of 1.4348 at 176° F. (80° C.), and an oil content of 0.6%.

The oil-solvent mixture or mother liquor displaced from the wax mass aforesaid was further diluted with ethylene dichloride to give a solution containing 20 parts by volume of oil-wax stock and 80 parts by volume of ethylene dichloride. This solution was then chilled to about 0° F., a portion of the wax crystallized therefrom, and the residual mother liquor displaced with 88° naphtha at 0° F., in the manner above described. The resulting washed wax, after removal of the naphtha, had an A. S. T. M. melting point of 119.5° F., a refractive index of 1.4374 at 176° F. (80° C.), and an oil content of 0.2%.

This substantially oil-free wax was then fractionated by sweating, the properties of the fractions being shown in Table I below.

Table I

| Cut No. | Final sweating temperature | Percent yield | A. S. T. M. melting pt. | Refractive index (80° C.) |
|---------|----------------------------|---------------|-------------------------|---------------------------|
| 1.....  | °F.                        |               | °C.                     |                           |
| 1.....  | 116                        | 38.7          | 112.5 (44.5)            | 1.4388                    |
| 2.....  | 116                        | 17.5          | 116.0 (46.3)            | 1.4390                    |
| 3.....  | 122                        | 23.4          | 120.5 (49.2)            | 1.4365                    |
| 4.....  | 128                        | 9.9           | 126.0 (52.3)            | 1.4358                    |
| 5.....  | 128                        | 10.5          | 133.0 (55.7)            | 1.4346                    |

By way of comparison, there is shown in Table II the properties of the wax fractions obtained by the sweating of a substantially oil-free commercial paraffin wax having an A. S. T. M. melting point of 122.5° F. (50.4° C.) and a refractive index of 1.4228 at 80° C., which was produced by sweating paraffin slack wax in the conventional manner.

Table II

| Cut No. | Final sweating temperature | Percent yield | A. S. T. M. melting pt. | Refractive index (80° C.) |
|---------|----------------------------|---------------|-------------------------|---------------------------|
| 1.....  | °F.                        |               | °F. °C.                 |                           |
| 1.....  | 114                        | 14.5          | 111.5 (43.8)            | 1.4250                    |
| 2.....  | 119                        | 21.0          | 116.5 (46.5)            | 1.4254                    |
| 3.....  | 124                        | 23.0          | 121.0 (49.6)            | 1.4260                    |
| 4.....  | 129                        | 16.1          | 125.5 (52.0)            | 1.4265                    |
| 5.....  | 134                        | 13.9          | 130.0 (54.0)            | 1.4276                    |
| 6.....  | 134                        | 11.5          | 136.5 (57.5)            | 1.4285                    |

Referring now to Fig. 1 of the drawings there is illustrated graphically the novel relationship between the melting points and refractive indices 75 of the wax fractions produced in accordance with

our process, as compared with the fractions resulting from the sweating of the commercial paraffin wax. Refractive indices at 80° C., are shown as the abscissae and the melting points as determined by the A. S. T. M. method No. 5 D-87-22 are shown as ordinates.

Upon determining the refractive index-melting point relationship for a large number of common waxes and paraffin hydrocarbons, it was found that substantially all of the waxes and hydrocarbons fell within a band or zone defined by 10 diagonal lines whose equations are

$$n = 1.4000 + 0.00044T \text{ and } n = 1.4070 + 0.00044T,$$

respectively, wherein "n" is the refractive index at 15 80° C., and "T" is the A. S. T. M. melting point. The series of diagonal lines shown in Fig. 1 are drawn parallel to the line whose equation is

$$n = 1.4000 + 0.00044T,$$

and differ from one another in their refractive index intercepts by 0.005.

It will be noted from curve A, which represents the wax fractions as obtained in accordance with Example 1 described hereinabove, that as the melting point increases the refractive index decreases, whereas in curve B, which represents the wax fractions obtained by sweating the commercial paraffin wax of Example 2 (given below), it will be seen that the relationship is reversed, i. e., 25 with increase in melting point the refractive index also increases. Wax fractions on curve B, corresponding substantially in melting point with those on curve A, fall within the band defined by 30 lines whose equations are  $n = 1.4035 + 0.00044T$  and  $n = 1.4058 + 0.00044T$  respectively, the maximum difference in the abscissae intercept values being 0.0023, whereas the wax fractions on curve A fall within the band defined by the lines whose 35 equations are

$$n = 1.410 + 0.00044T \text{ and } n = 1.4192 + 0.00044T$$

respectively, the maximum difference in the abscissae intercept values being 0.0092.

The following examples, in conjunction with the curves shown in Figures 2 and 3 of the drawings, will further illustrate the results which may be obtained in accordance with our invention.

*Example 2.*—An East Texas paraffin distillate was distilled to yield a wax-bearing fraction comprising the 1st 40% of the distillate. From this fraction there was separated at a temperature of about -20° F., and in accordance with the 1st procedure set forth in Example 1, a substantially oil-free wax having an A. S. T. M. melting point of 93° F. (33.9° C.) and a refractive index of 1.4205 at 176° F. (80° C.). This was fractionated by sweating to give a series of cuts having the properties indicated in Table III, the relationship of the refractive indices to the melting points being shown by curve C of Fig. 2 of the drawings.

Table III

| Cut No. | Percent yield     | A. S. T. M. melting pt. | Refractive index (80° C.) |
|---------|-------------------|-------------------------|---------------------------|
| 1.....  | °F. °C.           |                         |                           |
| 1.....  | 14.5 83.0 (28.5)  | 1.4197                  |                           |
| 2.....  | 52.1 88.5 (31.5)  | 1.4203                  |                           |
| 3.....  | 33.4 102.0 (39.1) | 1.4221                  | 70                        |

*Example 3.*—The initial substantially oil-free wax produced in accordance with Example 2, having an A. S. T. M. melting point of 93° F. (33.9° C.) and a refractive index of 1.4205 at 176° 75

F. (80° C.), was distilled under reduced pressure (10 m/m) to yield a bottoms or residual wax comprising 33.8% of the charge and having an A. S. T. M. melting point of 114.8° F. (46.0° C.) 5 and a refractive index of 1.4269 at 176° F. (80° C.). This residual wax was fractionated by sweating to give a series of cuts having the properties indicated in Table IV, the relationship of the refractive indices to the melting points being 10 shown by curve D of Fig. 2 of the drawings.

Table IV

| 15 | Cut No. | Percent yield | A. S. T. M. melting pt.   | Refractive index (80° C.) |
|----|---------|---------------|---------------------------|---------------------------|
| 1  |         | 17.2          | ° F. ° C.<br>108.0 (42.3) | 1.4263                    |
| 2  |         | 41.1          | 114.0 (45.5)              | 1.4266                    |
| 3  |         | 32.5          | 119.5 (48.5)              | 1.4266                    |
| 20 | 4       | 8.2           | 126.0 (52.3)              | 1.4270                    |

*Example 4.*—From a wax-bearing intermediate lubricating distillate having a Saybolt universal viscosity of 54 seconds at 210° F., and an A. P. I. gravity of 25.5 at 60° F., there was produced by the first step of the "displacement" method aforementioned, at a separation temperature of about 60° F., a substantially oil-free wax having an A. S. T. M. melting point of 153.8° F. (67.7° C.), 25 a refractive index of 1.4348 at 176° F. (80° C.), and an oil content of 0.4%. This substantially oil-free wax was subsequently sweated at a temperature of from 151° F. to 162° F., and a series of cuts were produced having the properties indicated in Table V, the relationship of refractive indices to melting points being shown by curve E of Figure 2 of the drawings.

Table V

| 40 | Cut No. | Percent yield | A. S. T. M. melting pt.   | Refractive index (80° C.) |
|----|---------|---------------|---------------------------|---------------------------|
| 45 | 1       | 54.3          | ° F. ° C.<br>150.0 (65.5) | 1.4348                    |
| 2  |         | 20.1          | 153.5 (67.5)              | 1.4340                    |
| 3  |         | 18.0          | 156.5 (69.2)              | 1.4342                    |
| 4  |         | 7.6           | 160.5 (71.5)              | 1.4349                    |

*Example 5.*—The efflux or mother liquor obtained by displacement from the wax of Example 50 4 was chilled to about 0° F., and a second wax fraction was crystallized therefrom and washed free of oil. This wax fraction had an A. S. T. M. melting point of 119.5° F. (48.7° C.), a refractive index of 1.4374 and an oil content of 0.3%. Upon sweating this wax fraction at a temperature of from 107° F. to 127° F., there was produced a series of cuts having the properties indicated in Table VI, the relationship of the refractive indices to the melting points being illustrated by 55 curve F of Fig. 2 of the drawings.

Table VI

| 65 | Cut No. | Percent yield | A. S. T. M. melting pt.   | Refractive index (80° C.) |
|----|---------|---------------|---------------------------|---------------------------|
| 70 | 1       | 38.7          | ° F. ° C.<br>112.5 (44.7) | 1.4288                    |
| 2  |         | 17.5          | 118.0 (46.7)              | 1.4280                    |
| 3  |         | 22.4          | 120.5 (49.2)              | 1.4285                    |
| 4  |         | 9.0           | 126.0 (52.3)              | 1.4288                    |
| 5  |         | 10.5          | 133.0 (56.0)              | 1.4295                    |

*Example 6.*—From a wax-bearing petrolatum stock having a Saybolt universal viscosity of 69 75 seconds at 210° F., and an A. P. I. gravity of 27.5°

at 60° F., there was produced, substantially in accordance with the 1st step of the "displacement" method described hereinbefore, at a separation temperature of about 65° F., a substantially oil-free wax having an A. S. T. M. melting point of 156° F. (69° C.), a refractive index of 1.4413 at 176° F. (80° C.), and an oil content of 0.4%. This substantially oil-free wax was fractionated by sweating at a temperature of from 147° F. to 162° F., and a series of cuts were produced having the properties indicated in Table VII, the relationships of the refractive indices to the melting points being shown by curve G of Fig. 2 of the drawings.

Table VII

| 15 | Cut No. | Percent yield | A. S. T. M. melting pt.   | Refractive index (80° C.) |
|----|---------|---------------|---------------------------|---------------------------|
| 1  |         | 23.0          | ° F. ° C.<br>152.5 (67.0) | 1.4418                    |
| 2  |         | 27.7          | 155.0 (68.3)              | 1.4414                    |
| 3  |         | 39.1          | 157.5 (69.7)              | 1.4410                    |
| 4  |         | 10.2          | 162.0 (72.2)              | 1.4405                    |

*Example 7.*—The efflux or mother liquor obtained by displacement from the wax of Example 8 was chilled to about 5° F., and a second wax fraction was crystallized therefrom and washed free of oil. This wax fraction had an A. S. T. M. melting point of 121.0° F. (49.6° C.), a refractive index of 1.4478 at 176° F. (80° C.), and an oil content of 0.3%. Upon sweating this wax fraction at a temperature of from 109° F. to 149° F., there was produced a series of cuts having the properties indicated in Table VIII, the relationship of the refractive indices to the melting points being shown in curve H of Fig. 2 of the drawings.

Table VIII

| 25 | Cut No. | Percent yield | A. S. T. M. melting pt.   | Refractive index (80° C.) |
|----|---------|---------------|---------------------------|---------------------------|
| 1  |         | 30.3          | ° F. ° C.<br>112.0 (44.5) | 1.4490                    |
| 2  |         | 28.8          | 117.0 (47.2)              | 1.4488                    |
| 3  |         | 29.9          | 124.0 (51.1)              | 1.4476                    |
| 4  |         | 11.0          | 133.5 (56.3)              | 1.4460                    |

*Example 8.*—From a fraction of a paraffin distillate having a Saybolt universal viscosity of 90 seconds at 100° F., and an A. P. I. gravity of 30.5° at 60° F., there was produced, substantially in accordance with the 1st step of the "displacement" method described in connection with Example 1, at a separation temperature of about 40° F., a substantially oil-free wax having an A. S. T. M. melting point of 132° F. (55.5° C.), a refractive index of 1.4286 at 176° F. (80° C.), and an oil content of 0.6%. This substantially oil-free wax was fractionated by sweating at a temperature of from 122° F. to 133° F., and a series of cuts was produced having the properties indicated in Table IX, the relationship of the refractive indices to the melting points being shown by curve I of Fig. 3 of the drawings.

Table IX

| 40 | Cut No. | Percent yield | A. S. T. M. melting pt.   | Refractive index (80° C.) |
|----|---------|---------------|---------------------------|---------------------------|
| 1  |         | 32.5          | ° F. ° C.<br>127.5 (50.3) | 1.4285                    |
| 2  |         | 35.9          | 131.5 (55.2)              | 1.4285                    |
| 3  |         | 31.6          | 138.0 (59.0)              | 1.4289                    |

Example 9.—The efflux or mother liquor obtained by displacement from the wax of Example 8 was chilled to about 0° F., and a second wax fraction was crystallized therefrom and washed free of oil. This wax fraction had an A. S. T. M. melting point of 106.5° F. (41.4° C.), and a refractive index of 1.4262 at 176° F. (80° C.). Upon sweating this wax fraction at a temperature of from 102° F. to 122° F., there was produced a series 10 of cuts having the properties indicated in Table X, the relationship of the refractive indices to the melting points being shown by curve J of Fig. 3 of the drawings.

Table X

| 15 | Cut No. | Percent yield | A. S. T. M. melting pt.  | Refractive index (80° C.) |
|----|---------|---------------|--------------------------|---------------------------|
| 20 | 1       | 9.4           | ° F. ° C.<br>98.0 (36.7) | 1.4277                    |
|    | 2       | 75.3          | 106.0 (41.1)             | 1.4256                    |
|    | 3       | 12.1          | 115.0 (46.1)             | 1.4258                    |
|    | 4       | 3.2           | 121.5 (50.7)             | 1.4264                    |

Example 10.—Approximately 50% of the initial oil-free wax of Example 4 and 50% of the initial oil-free wax of Example 5 were admixed to form a homogeneous product having an A. S. T. M. melting point of 146.0° F. (63.3° C.), and a refractive index of 1.4367 at 176° F. (80° C.). This product was fractionated by sweating at a temperature of from 115° F. to 160° F., and there was produced a series of cuts having the properties indicated in Table XI, the relationship of the refractive indices to the melting points being shown by curve K of Fig. 3 of the drawings.

Table XI

| 40 | Cut No. | Percent yield | A. S. T. M. melting pt.   | Refractive index (80° C.) |
|----|---------|---------------|---------------------------|---------------------------|
|    | 1       | 6.3           | ° F. ° C.<br>130.0 (54.5) | 1.4377                    |
| 45 | 2       | 47.7          | 143.0 (61.7)              | 1.4366                    |
|    | 3       | 33.1          | 148.0 (64.5)              | 1.4361                    |
|    | 4       | 12.9          | 158.0 (70.0)              | 1.4355                    |

It will be seen from the above examples that, in general, the wax cuts or fractions produced in accordance with our invention are characterized by the fact that as the melting points increase, the refractive indices decrease, which relationship is not characteristic of the waxes produced by the conventional sweating processes applied to the common paraffin waxes, for example, the sweating of commercial paraffin wax. It will further be seen that the wax fractions produced in accordance with our invention differ from one another in their refractive index intercepts to a much greater extent than do those of the wax fractions produced by the sweating of known waxes, for example, commercial paraffin wax. In the equations of the type relating refractive index to melting point, i. e.,  $n = x + 0.00044T$ , where "n" denotes the value of the refractive index, "T" denotes the melting point in °C., and "x" denotes refractive index intercept values, the difference in the value of "x" for different wax fractions, produced in accordance with our invention, may be of the order of 0.0025, 0.005, 0.0075 and 0.01 or more, whereas the differences in such values for the known waxes are usually of the order of 0.002 or less.

Furthermore, the wax fractions produced in accordance with our invention differ from the

common hydrocarbon waxes of corresponding melting points in that they possess much higher boiling points than the corresponding waxes heretofore known; their refractive indices are substantially higher than those of the corresponding known waxes; their molecular weights are much higher than those of the corresponding known waxes, and they differ from the known waxes in other properties such as hardness, tackiness and plasticity.

We have found, as another aspect of our invention, that in order to produce the highest yield of high melting point wax of desired properties, and the highest yield of low melting point wax of desired properties, from a mixture of hydrocarbon waxes, it is preferable to effect a separation of substantially all of the oil from the wax and to separate or segregate the higher melting waxes, as one or more fractions, from the lower melting waxes, as one or more fractions, prior to subjecting such wax to fractionation by sweating. This separation or segregation may be effected by the "displacement" process aforementioned, or by other methods involving, for example, solvent treatment, recrystallization or distillation. This aspect of our invention may be illustrated by the following example.

From a wax-bearing lubricating oil distillate there was produced by a single "displacement" operation, a substantially oil-free wax fraction having an A. S. T. M. melting point of 146° F., and containing high and low melting point waxes. This fraction was then sweated to produce a wax cut having a melting point of 150° F. and the yield obtained was of the order of 33% by weight, based on the total quantity of wax separated from the distillate.

Upon subjecting the same wax-bearing distillate to a double or 2 stage "displacement" operation at two different temperatures, whereby the higher melting waxes were segregated in the 1st fraction and the lower melting waxes in the 2nd fraction, there was produced two substantially oil-free fractions having A. S. T. M. melting points of 153.8° F. and 119.5° F., respectively. The fraction having the higher melting point was then sweated to produce a wax cut having a melting point of 150° F. and the yield obtained was of the order of 54%, by weight, based on the total quantity of wax separated from the distillate.

It will be seen, from the above example, that the yield of 150° F. melting point wax was markedly increased by separating the wax initially present in the distillate into at least two fractions, prior to sweating that fraction containing the higher melting point waxes. Substantially the same method may be applied to the recovery of high yields of low melting wax, when the initial stock comprises a mixture of the waxes of varying melting points.

Our method of treatment may be applied to a variety of waxes or wax-bearing oils, for example, viscous wax-bearing distillates and residuums, and particularly wax-bearing oils having Saybolt universal viscosities at 210° F., within the range of from about 40 seconds to about 400 seconds, to produce substantially oil-free waxes having the novel relationship between refractive indices and melting points hereinbefore set forth. The step of fractionation by sweating may be carried on at any suitable temperature, and preferably within the range of from about 85° F. to about 180° F.

While, in general, we have described our step of segregation or "displacement" to produce sub-

stantially oil-free wax mixtures, utilizing ethylene dichloride and 88° naphtha as solvents, we do not intend to limit ourselves thereto, but may employ any conventional dewaxing solvent or solvent mixture, for example, naphtha, alcohol, acetone, acetone-benzol, and the like, as well as the liquefied normally gaseous hydrocarbons such as ethane, propane, butane, pentane and the like, or mixtures thereof.

10 Herein, and in the appended claims, the term "substantially oil-free wax" is to be understood to comprehend wax which contains less than substantially 2% by weight of oil, as determined in accordance with the method disclosed in the co-pending application of S. W. Ferris, Serial No. 4,157, filed January 30, 1935 and entitled "Treatment of wax".

What we claim is:

1. In a process for treating a hydrocarbon oil-wax mixture, the steps which comprise segregating from said mixture, a fraction containing the higher melting wax components thereof substantially free of oil and a fraction containing the lower melting wax components thereof substantially free of oil and subjecting at least one of said fractions to sweating.

2. In a process for treating a hydrocarbon oil-wax mixture containing higher melting and lower melting wax components, the steps which comprise forming a homogeneous mixture of oil, wax

and a solvent for the oil, reducing the temperature of the mixture to cause higher melting wax components to crystallize, separating the mixture of oil, solvent and lower melting wax components from the crystallized wax and thereby producing a substantially oil-free higher melting wax fraction and subjecting said higher melting fraction to sweating.

3. In a process for treating a hydrocarbon oil-wax mixture containing higher melting and lower melting wax components, the steps which comprise forming a homogeneous mixture of oil, wax and a solvent for the oil, reducing the temperature of the mixture to cause higher melting wax components to crystallize, separating the mixture of oil, solvent and lower melting wax components from the crystallized wax to produce a substantially oil-free higher melting wax fraction, further cooling said separated mixture of oil, solvent and lower melting wax components to cause lower melting wax components to crystallize, separating the remaining oil-solvent mixture from said crystallized lower melting wax components and thereby producing a substantially oil-free lower melting wax fraction, and subjecting at least one of said substantially oil-free wax fractions to sweating.

SEYMOUR W. FERRIS.

WILLARD F. HOUGHTON.

HENRY C. COWLES, JR.

30